

Feb. 12, 1924.

1,483,450

E. F. KENNEY

MAKING IRON AND TUBES

Filed Feb. 21, 1923

*Fig. 1.*



*Fig. 2.*



*Fig. 3.*



*Fig. 4.*



*Fig. 5.*



*Fig. 6.*



*Fig. 7.*



*Fig. 9.*



*Fig. 10.*



BY

INVENTOR  
Edward F. Kenney  
Geo. E. Thackray  
ATTORNEY

*Fig. 8.*



Patented Feb. 12, 1924.

1,483,450

# UNITED STATES PATENT OFFICE.

EDWARD F. KENNEY, OF PHILADELPHIA, PENNSYLVANIA.

## MAKING IRON AND TUBES.

Application filed February 21, 1923. Serial No. 620,458.

To all whom it may concern:

Be it known that I, EDWARD F. KENNEY, a citizen of the United States, and a resident of the city of Philadelphia, county of Philadelphia, and State of Pennsylvania, have invented certain new and useful Improvements in Making Iron and Tubes; and I do hereby declare the following to be a full, clear, and exact description of the invention, 10 such as will enable others skilled in the art to which it appertains to make and use the same.

My invention relates to making wrought iron which is rolled or hammered from a ball or loup, into plates or bars and then successively cutting and piling said plates or bars; arranging the plates, heating and rolling the same in different directions while welding the various layers, so as to produce 20 a product which is stronger in all directions than heretofore.

My invention is particularly adapted for use in making pipes or boiler tubes as practically all of the tests prescribed for charcoal 25 boiler tubes test the metal in circumferential directions, and such tests are very severe on material like the usual knobbled charcoal iron and wrought iron otherwise produced, for the reason that in prior practice the slag 30 or cinder which is originally contained in the mass is all rolled into threads or fibers parallel to the rolling direction making the rolled material weak in a lateral direction or circumferentially of the tube formed 35 therefrom.

In order to obviate this I take a ball or loup of wrought iron which may be formed in a charcoal knobbling fire, by busheling scrap, or puddling, or in other ways, which 40 ball is composed of a large number of granules of wrought iron in a heated and plastic condition, secured together by contact coherence of their surfaces and between and around these granules are layers of slag, or 45 cinder and oxides.

I take this ball or loup, and forge it into a bloom which is of approximately rectangular cross section and then roll it longitudinally to produce a muck bar and then 50 cut the muck bar into convenient lengths and form a pile therefrom; I then heat and roll this pile in a direction transverse to or substantially at right angles to the first rolling of the bloom, thereby welding the various 55 layers together and forming a plate or wide bar. I then shear this plate crosswise into

pieces of widths necessary to make a tube sheet or skelp of any width desired and pile these again, heat and roll them longitudinally, while welding the various layers, this 60 rolling being in a direction substantially at right angles to the second direction of rolling, and consequently substantially parallel to the first rolling direction of the bloom into muck bar. 65

Tests in different directions have been made on tubes manufactured from skelp produced in the manner indicated by my invention, which show that these meet all tests 70 much better than tubes made by the prior practice.

One of the advantages of my method is that only one width of muck bar need be produced, thus requiring only one set of rolls and thereby eliminating roll changes. 75

Another advantage is that the material for the final piling to produce all widths of skelp can be cut from one plate or wide bar by shearing the same crosswise to any widths necessary, which permits such plate or wide 80 bar to be kept in stock and the skelp mill maintained in continuous operation without running the muck bar mill at the same time.

Another advantage is that the skelp so made is strong in all directions, thus obviating rejections and facilitating its use. 85

My invention is applicable to producing wrought iron in various forms or shapes, including skelp for the production of boiler tubes and the drawings herewith are merely 90 diagrammatic thereof.

Having thus given a general description of my invention, I will now, in order to make the matter more clear, refer to the annexed sheet of drawings, which form part 95 of this specification, and in which like characters refer to like parts:—

Figure 1 is a perspective view showing a ball or loup of wrought iron produced in a charcoal knobbling fire or otherwise; Figure 2 is a perspective view of a bloom which is preferably hammered from the ball; Figure 3 is a portion of a muck bar rolled from the bloom of Figure 2; Figure 4 is a perspective view of the first pile 100 formed from the muck bar after it has been cut to lengths and piled; Figure 5 is a perspective view of a part of a plate or wide bar rolled in a lateral direction from the pile of Figure 4; Figure 6 is a view of a pile formed from strips cut laterally of the plate or wide bar of Figure 5; Figure 7 is 105 110

1 perspective view of tube skelp rolled from the pile of Figure 6 in a longitudinal direction; Figure 8 are cross sections of tube skelp which may either have scarfed or square edges as illustrated; Figure 9 is a perspective view of a portion of skelp, bent prior to forming a welded tube therefrom and Figure 10 is a perspective view of a part of a finished boiler tube which has been 10 welded in the usual welding rolls or otherwise.

Referring now to the characters of reference on the drawings:—1 is a ball of wrought iron which may be made in a charcoal knobbling fire, by busheling scrap, puddling or otherwise; 2 is a bloom which has been forged from the ball 1; 3 is a muck bar which has been rolled from the bloom 2, by passing it when heated through rolls, the 20 direction of rolling being indicated by the line A—B, after which it is cut into pieces 4, as shown by the dotted lines indicating the ends 5, and piled to form the pile 6, this pile is then heated and welded by being 25 passed through reducing rolls in the lateral direction C—D which forms the plate or wide bar 7; this plate is then cut transversely as indicated by the dotted lines 9 into the pieces 8 and these pieces may be any width 30 desired to produce skelp of proper size from which to form a tube of any desired diameter. These pieces 8, are then laid together to form the pile 10 which pile is again heated and welded by being rolled in the direction F—G to form the skelp 11 and this skelp 11 may be cut as indicated at 13 in lengths 12 suitable for forming pipes or 35 tubes therefrom. The skelp 11 may be rolled or otherwise provided, with beveled or scarfed edges 14, or it may have square edges as indicated at 17. Preparatory to welding the tube, the length 12 of the skelp is heated and bent into the form 15 after which it is 40 heated to welding temperature and passed through welding rolls and its edges are welded together forming the tube 16.

A loup or ball of knobbled charcoal or wrought iron consists of a plurality of cohering granules of iron and between or 50 around them are layers of slag or cinders, and oxides, and in accordance with previous practice, the bloom is hammered therefrom and elongated in one direction producing elementary fibers in the metal and also elementary fibers of slag or cinder, or oxides 55 between the fibers of metal which are further and greatly elongated by successive longitudinal rollings producing lateral discontinuities or breaks in the metal, as the 60 fibers thereof are separated by fibers of the occlusions, so that skelp so made while strong longitudinally is weak laterally, thus resembling a rope of wires and when skelp is formed into a tube it will not stand the 65 circumferential tests applied to it nor the

actual tests of the various uses to which it will be subjected.

I obviate this by my invention, as above described by piling heating and rolling in various directions, thereby welding the various layers together, so that the slag, etc., no longer forms longitudinal breaks or fibers between the fibers of the metal but is more uniformly distributed in very small particles or thin laminæ, thus producing iron 75 which is stronger in all directions.

Although I have, for the purpose of simplicity of illustration and description, described my invention in connection with making boiler tubes I wish it to be understood that it also relates to making wrought iron bars, plates and other shapes by successive rollings in different directions, the bars being cut between the rollings and placed together to form piles which are heated preparatory to rolling, the last rolling being 85 preferably in a direction longitudinal of the last pile.

Although I have shown and described my invention in considerable detail, I do not 90 wish to be limited to the exact and specific details thereof, as shown and described, but may use such modifications in, substitutions for, or equivalents thereof as are embraced with the scope of my invention, or as 95 pointed out in the claims.

Having thus described my invention, what I claim and desire to secure by Letters Patent is:—

1. The method of forming tube skelp, 100 consisting of rolling a wrought iron bloom, and then successively cutting, piling, heating and rolling the piles in different directions, while welding the layers together.

2. The method of forming tube skelp, 105 consisting of longitudinally rolling a wrought iron bloom, then successively cutting, piling, heating and rerolling bars from the piles formed therefrom, thereby welding the layers together, said rolling being 110 done both longitudinally and transversely of the original axis, thereby producing skelp strong in all directions.

3. The method of making wrought iron 115 which consists in taking a heated ball thereof, compressing the same laterally while extending it longitudinally, thereby forming a bloom, then reducing the cross section of said bloom, while extending it longitudinally, thereby forming a bar, then cutting said 120 bar into lengths and placing them together to form a pile, then heating said pile and reducing its cross section while extending it transversely in a direction different from the first extensions, thereby forming a wider 125 bar, then cutting a plurality of bars transversely therefrom, then placing said bars together to form a pile, then heating the pile and reducing its cross section while extending it longitudinally in a direction similar 130

to that of the first extensions above described.

4. The steps in the method of making iron tubes which consists in taking a heated ball 5 or loup of wrought iron intermingled with slag and oxides, forging and compressing the same to a bloom of approximately rectangular cross section, then rolling said bloom longitudinally, thereby producing a 10 muck bar, then cutting said muck bar into predetermined lengths and placing said lengths together to form a pile, then heating said pile and rolling it in a direction transverse to the previous direction, thereby 15 forming a wider bar, then transversely cutting strips of predetermined width therefrom, then placing said strips together to form a pile, then heating said pile and rolling the same longitudinally to form a tube 20 skelp.

5. The method of forming a tube, consisting of longitudinally rolling a wrought iron bloom, then successively cutting, piling, heating and rerolling bars from the piles 25 formed therefrom, said rolling being done both longitudinally and transversely of the original axis, thereby producing skelp strong in all directions, then bending said skelp with its longitudinal edges overlap-

ping, then heating it to welding temperature and then welding said edges together in welding rolls or otherwise to form a tube. 30

6. The method of forming a tube which consists in taking a heated ball or loup of wrought iron intermingled with slag and 35 oxides, forging and compressing the same to a bloom of approximately rectangular cross section, then rolling said bloom longitudinally, thereby producing a muck bar, then cutting said muck bar into predetermined 40 lengths and placing said lengths together to form a pile, then heating said pile, and rolling it in a direction transverse to the previous direction, thereby forming a wider bar, then transversely cutting strips of predetermined width therefrom, then placing 45 said strips together to form a pile, then heating said pile and rolling the same longitudinally to form a tube skelp, then bending said skelp with its longitudinal edges overlapping, then heating it to welding temperature, and then welding said edges together in welding rolls or otherwise to form 50 a tube.

In witness whereof I hereunto affix my 55 signature.

EDWARD F. KENNEY.